

E. F. GOLTRA, T. S. MAFFITT, J. D. DANA & R. W. ERWIN.  
APPARATUS FOR CLEARING CLAYEY ORES.

1,288,404.

APPLICATION FILED JAN. 5, 1914.

Patented Dec. 17, 1918.

4 SHEETS—SHEET 1.



Attest:  
Chas. A. Becker  
S. F. Linhardt.

Inventors:  
E. F. Goltra, T. S. Maffitt,  
J. D. Dana and R. W. Erwin,  
by John H. Brumley  
Their Attorney

E. F. GOLTRA, T. S. MAFFITT, J. D. DANA & R. W. ERWIN.

## APPARATUS FOR CLEARING CLAYEY ORES.

APPLICATION FILED JAN. 5, 1914.

1,288,404.

Patented Dec. 17, 1918.

4 SHEETS—SHEET 2.



Attest:  
Chas. A. Becker  
G. F. Reinhardt

Inventors:  
E. F. Gottra, F. S. Maffitt,  
J. D. Dana and R. W. Erwin  
by John N. Brumley, Their Attorney.

E. F. GOLTRA, T. S. MAFFITT, J. D. DANA & R. W. ERWIN.  
APPARATUS FOR CLEARING CLAYEY ORES.

APPLICATION FILED JAN. 5, 1914.

APPLICATION FILED JAN. 5, 1914.

1,288,404.

Patented Dec. 17, 1918.

4 SHEETS—SHEET 3.



St. Leon:

Inventors:  
E. F. Gottes, J. B. Maffitt,  
J. H. Harr, and R. W. Ervin,  
by John A. Brumaga, their Attorney.

E. F. GOLTRA, T. S. MAFFITT, J. D. DANA & R. W. ERWIN.

## APPARATUS FOR CLEARING CLAYEY ORES.

APPLICATION FILED JAN. 5, 1914.

1,288,404.

Patented Dec. 17, 1918.

4 SHEETS—SHEET 4.



Attest: + 9

Chas. A. Becker,  
J. F. Linhardt.

Inventors  
E. G. Gollva, J. S. Haffill,  
J. D. Dana and R. W. Erwin  
by John N. Brunning their Attorney

# UNITED STATES PATENT OFFICE.

EDWARD F. GOLTRA, THOMAS S. MAFFITT, AND JESSE D. DANA, OF ST. LOUIS, MISSOURI, AND ROBERT W. ERWIN, OF WAUKON, IOWA, ASSIGNEES, BY MESNE ASSIGNMENTS, TO MISSISSIPPI VALLEY IRON COMPANY, OF WILMINGTON, DELAWARE, A CORPORATION OF DELAWARE.

## APPARATUS FOR CLEARING CLAYEY ORES.

1,288,404.

Specification of Letters Patent. Patented Dec. 17, 1918.

Application filed January 5, 1914. Serial No. 810,531.

To all whom it may concern:

Be it known that we, EDWARD F. GOLTRA, THOMAS S. MAFFITT, JESSE D. DANA, and ROBERT W. ERWIN, citizens of the United States, said GOLTRA, MAFFITT, and DANA residing at St. Louis, State of Missouri, and said ERWIN residing at Waukon, Iowa, have invented new and useful Improvements in an Apparatus for Clearing Clayey Ores, of which the following is a specification.

This invention relates to apparatus for clearing ore of its gangue, and more particularly to apparatus for clearing ores containing clay as a gangue.

Some ores, such as brown hematite and certain ores of copper, contain a large percentage of clay and sometimes silica as a gangue. These ores exist as nodules and boulders of various sizes in the clay beds, and the clay and silica, such as flint, stone, gravel and sand, is often found inside of the lumps or boulders. Now this gangue must be separated from the ore before it can be used economically in a blast furnace.

In U. S. Patents Nos. 957,157, granted May 3, 1910, and 961,121, granted June 14, 1910, are described a process for clearing such clayey ore of its gangue. The process as described in said patents may be briefly summed up as follows: The ore and its gangue are heated at a temperature and for a period sufficient to render the gangue brittle and easily separable from the ore; the ore and its gangue are tumbled to shake loose the gangue from the ore, and the ore and gangue are subjected to a strong air blast so as to sweep, clean and remove the gangue from the ore.

While the air cleaning process of said patents produces a merchantable ore well suited for a blast furnace, and while this air cleaning process will free the ore of substantially all of its clay gangue, it will not separate the rock, flint, gravel and sand from the ore to a sufficient extent. As stated above, this silica occurs in combination with clay as a gangue, and often occurs inside of the lumps or boulders of ore.

One of the objects of this invention therefore is to refine the apparatus described in the above patents so as to render it more efficient, so as to clear the ore of all of its

gangue, whether of a clay or siliceous character, and so as to avoid losses of ore.

Another object is to adapt the apparatus for various ores having characteristics permitting its utilization, more particularly various ores containing clay as a gangue and occurring in the form of nodules in the clay, and containing considerable moisture both free and combined.

Further objects will appear from the detail description taken in connection with the accompanying drawings in which:

Figure 1 is a diagrammatical plan view of an apparatus illustrating the process embodying this invention,

Fig. 2 is a profile or elevation also in diagrammatical form,

Fig. 3 is an enlarged diagrammatical detail profile or elevation,

Fig. 4 is another enlarged diagrammatical detail profile or elevation showing the second converter,

Fig. 5 is a plan showing the third converter,

Fig. 6 is a profile or side elevation partly in section, of this third converter,

Fig. 7 is a detail end elevation, showing the outlet door,

Fig. 8 is a detail end elevation of the inlet end,

Fig. 9 is a section on the line 9—9 Fig. 8,

Fig. 10 is an enlarged detail section on the line 9—9 Fig. 8, and

Fig. 11 is an enlarged detail section on the line 11—11 Fig. 9.

The apparatus generally stated consists of three converters designated generally by A, B and C.

The first converter comprises a cylinder 10 having rings 11 resting on rolls 12 and 129 on pillars 13, and 14. The cylinder is positioned on an incline, and the upper set of rings 11 and rolls 129 forms an end thrust bearing to support the cylinder against end movement. This cylinder is constructed of boiler iron and may be about 125 feet long and 10 feet in diameter. It is lined for about one-third of its length from its lower end with fire brick or other suitable material, while the unlined part has a series of inwardly projecting shelves or lifters extending therealong. The upper end of the

cylinder projects into a stationary hopper casing 16 connecting with a hopper 17, which hopper receives the ore from stationary grids 18 which in turn receive the ore from the mine. The grids are spaced any suitable distance so as to allow the ore below a certain size to pass therethrough; thus in this particular instance these grids are spaced from 12 to 14 inches apart so as to 5 allow everything under 14 inches to pass into the hopper 17. This hopper is provided with two hinged valve plates 20 and 21 placed in series to prevent the gases in the converter from entering the hopper. The 10 casing 16 is connected with a stack 22 through a fan 23 driven by a motor 24. This fan will cause a draft from the lower to the upper end of the cylinder and up the stack 22. The lower end of the cylinder 15 projects into a casing 25 which is provided with rolls so as to be movable longitudinally of the cylinder along a track 26, to allow for expansion and contraction of the cylinder. A pulverized coal burner 27 receives the coal from a bin 28 and an air 20 blast from a fan or pump 29, and this coal is blown in a pulverized condition into the lower end of the cylinder 10. The cylinder is provided with a toothed ring 30 meshing 25 with a pinion 31 driven by a suitable motor.

The ore is discharged from the cylinder 10 on shaking or reciprocating grids 35, which in this particular case discharge everything below  $2\frac{1}{2}$  inches into a chute 36, 30 while the oversize discharges into a crusher 37, which may be of the gyratory type, and which crusher reduces the material to  $2\frac{1}{2}$  inches. The chute 36 from the reciprocating grids, and the chute 38 from the crusher 35 discharge into an elevator 39, which elevates the material and discharges it into a sizing screen or trommel 40. This trommel sizes the material in this particular instance to three sizes. The fine material passes by a 40 chute 41 to a tailings bin 42, the second sized material passes by a chute 43 to a belt conveyer 44, discharging into the ore bin 45, and the oversize or coarse material passes onto a picking belt 46 where it is hand-45 picked and the picked ore discharged onto the conveyer 44 and hence taken to the ore bin 45. The hopper 47 for the tailings bin 42 extends upwardly underneath the belt 46 so as to receive the flint etc. picked from the belt.

The material from the bin 45 is taken to the second converter B which is shown in detail and enlarged in Fig. 4. This second converter is of substantially the same construction as the first converter A and is operated in substantially the same manner. It consists in this particular instance of an inclined cylinder 50 about 125 feet long and 8 feet in diameter. It is however lined for a 60 little over three fourths of its length from

its lower end with fire brick or the like, while the unlined part is provided with inwardly projecting shelves extending therealong. This cylinder is supported by rings 51 on rolls 52 and 520 on pillars 53 and 54. 70 The center set of rings 51 and rolls 520 in this case also form a thrust bearing. The upper end of the cylinder extends into a casing 56 which is connected to an exhaust fan 57 discharging into a dust collector 58 75 and from there into a stack 69. This dust collector may be of any suitable form and may be provided with inclined shelves 59 placed in staggered relation so as to separate the dust from the air before it is discharged into the 80 stack. An outlet 60 is provided for this dust collector. A conveyer 61 conveys the ore from the bin 45 to the casing 56 and thence to the cylinder 50. The lower end of the cylinder projects into a casing 62 provided 85 with rolls and adjustable lengthwise of the cylinder along a track 63. A pulverized coal burner 64 receives coal from a bin 65 and air from a blower or pump 66, and this burner blows the pulverized coal into the 90 lower end of the cylinder. The cylinder is provided with a toothed ring 67 meshing with a pinion 68 driven by a suitable motor.

The material as it leaves the second converter is taken by an elevator 70 to a sizing 95 trommel 71 which in this case sizes the ore to two sizes. The oversize is taken by a conveyer 72 and discharged onto a picking belt 73 where the flint etc. are hand-picked, while the picked ore is discharged into the 100 bin 74. The ore on the conveyer 72 is subjected to a water spray 75 so as to cool down the material before it reaches the picking belt 73.

The undersize from the trommel 71 is 105 discharged into a hopper 76 and into the third converter C which will now be described. Referring more particularly to Figs. 5 to 11 inclusive, which show the third converter in detail, 77 designates a 110 cylinder of boiler iron provided with rings 78 resting on rolls 79 on pillars 80, and having a center thrust ring 81 coöperating with thrust rolls 82. This cylinder is provided with a toothed ring 83 meshing with a pinion 84 driven by a suitable motor. The cylinder for about one-half of its length from its upper end is of a comparatively large diameter, while the lower end is reduced as shown at 85 so as to form a comparatively long outlet of small diameter. Thus in a practical case, the cylinder is 60 feet long, has a large diameter of  $6\frac{1}{2}$  feet and a small diameter of  $3\frac{1}{2}$  feet.

The upper end of the cylinder makes an 125 airtight connection with an end plate 86 supported on a bracket 87, the end connection being made by a ring 88 on a reduced extension 89 of the cylinder pressed by springs 90 against the end plate 86. The 130

hopper 76 discharges through double valve casings 91 and 92, and a chute 93 extending through the plate 86, into the cylinder 77. The valve casings 91 and 92 are provided 5 with valves 94 and 95 respectively, suspended by links 98 from levers 97 pivoted on the hopper casings. These levers are pivoted in the valve casings by sleeves 99 making close fits with bearing lugs 100 of the 10 valve casings so as to make these joints air tight. The levers 97 are provided with weights 101. Links 102 are pivoted at their lower ends to the arms 97 and are provided at their upper ends with elongated slots en- 15 gaging cranks 103 on a shaft 104, which is driven from any suitable source of power. A pipe 105 projects into the cylinder and extends just through the bottom wall of the chute 93. This pipe 105 delivers crude oil 20 under a pressure of about 150 lbs. per square inch from a tank 106.

The lower end of the cylinder 77 is closed by a door 107 pivoted at its upper end to the frame 108 and held closed by strong springs 25 109. The door 107 has a cut out portion 110 in which is pivoted a small door 111 closed by weaker springs 112. Both doors bear against the end of the cylinder so as to form an airtight joint, but the lower door 30 111 is opened by the material passing out of the cylinder, the opening being however only sufficient to permit the ore to pass out. The function of the double door is that of a safety device, for if an explosion takes place 35 both doors will blow open and therefore furnish a large outlet for the exploded gases and thereby prevent damage to the converter.

A conveyer 115 takes the material from the third converter to a sizing trommel 116 40 which sizes the material to a series of sizes so that it can be conveniently operated upon by magnetic separators. The material on the conveyer 115 is passed underneath sprays 114 of cold water to quench the 45 same. The material from the sizing trommel is conveyed to magnetic separators indicated at 117. These magnetic separators separate the ore from the gangue, the ore being conveyed to a suitable ore bin such as 74 50 and the tailings discarded.

The coal is stored in a bin 120 from whence it is conveyed to a drier 121. From the drier the coal is taken by conveyers 122 and 123 to bins 28 and 65 respectively. In 55 the diagrams, 124 designates the power house and 125 and 126 designate tracks.

The operation will now be described, and in this operation we will take as a practical case, for the material operated upon, limonite or brown hematite containing a large 60 percentage of clay as a gangue, containing also siliceous gangue such as stone, quartz, gravel and sand, and containing both free and combined moisture.

The ore as mined is dumped on the grids

18 which, as described above, pass everything under 14 inches, the larger lumps being broken up, to pass into the first converter A. This first converter is rotated at a slow speed, the speed of revolution and the 70 incline being such that it takes about 45 minutes for the material to pass therethrough. The flame temperature at the lower end of the converter is maintained at about 2200° F., while the stack temperature, or 75 the temperature at the upper end of the converter, is maintained at about the boiling point of water. The exhaust fan creates a draft of about one-half ounce. A low pressure current of air is thus passed through 80 the drum, the air entering both with the pulverized coal and through the outlet passage in the casing 25. The material in passing through the first converter is subjected to a drying heat, and the operation performed in 85 this first converter is therefore a drying operation, whereby the material is freed of substantially all of its free moisture. During 90 its passage through the converter the ore and gangue, including the heavy boulders, which are as large as 14 inches, are lifted and tumbled around, and during this tumbling operation the heavy boulders will break up to some extent and break and disintegrate the ore and gangue, so that a crushing 95 operation is performed in this converter. Simultaneously the mass of ore and gangue is subjected to a gradually increasing temperature, as the temperature increases from the upper to the lower end of the converter, 100 and this ore and gangue will therefore be gradually dried out. This combined drying and tumbling operation will also render the ore friable, and will in addition separate, 105 i. e., shake loose some of the clay and other gangue, including the larger stone, mixed with the clay. It will be noted however that while a draft of air is passed through the cylinder of this first converter, the blast is not a strong blast, for its function is merely 110 a drying function; its function is not primarily to carry off any of the gangue, although some of the clay which has become free and very finely powdered will be incidentally carried off by the draft. The ore 115 as it is discharged from the first converter is at about 250° F., and this ore will have freed therefrom substantially all of its free moisture. The ore is therefore in a dry and friable condition so that it can be readily crushed. Some of the clay gangue, more especially the surface gangue surrounding the ore lumps, will be dried, loosened, and broken and ground, so that it, together with the sand may be separated from the rest by 120 a trommel, as hereinafter described.

The ore and gangue as discharged from the first converter is passed over the shaking grids 35 which pass everything below 2½ inches into the elevator 39, while the over- 130

size is sent to the crusher 37 and crushed down to  $2\frac{1}{2}$  inches, and discharged into the elevator 39. This elevator takes the ore and gangue to the sizing trommel 40 which sizes 5 the material in three sizes as follows: one-sixteenth inch and below, one-sixteenth inch to three-fourths inch, and three-fourths inch and over. It is found that the one-sixteenth and below consists mostly of sand and clay 10 and is very lean in ore. This size is therefore discharged directly into the tailings bin 42. The one-sixteenth to three-fourths is discharged directly into the ore bin 45 by means of the conveyer belt 44. The three- 15 fourths and over is discharged onto a picking belt 46 where the flint etc. are hand-picked, the picked ore passing into the ore bin. The purpose of the sizing between the second and third sizes is to facilitate the 20 hand picking, as it is found that most of the rock, flint and other siliceous material freed from the ore will be found in this size. This sizing of the ore therefore, first, discards the fines, consisting mostly of sand 25 and clay and containing very little ore, and second, throws only the larger sizes on the picking belt where the flint etc. may be readily hand-picked and discarded.

The material is taken from the ore bin 45 30 to the second converter B. This second converter is driven at such a speed, and the incline is such, that the material will pass through this converter in about 45 minutes. The flame temperature maintained at the 35 lower end of this converter is about  $3200^{\circ}$  F., while the temperature at the upper end is from  $400^{\circ}$  to  $500^{\circ}$  F. The exhaust fan in this case creates a strong blast through the converter cylinder of about  $1\frac{1}{2}$  ounces. 40 which blast will lift particles of sand one-sixteenth of an inch in diameter. As the material passes through the converter it is tumbled around, and at the same time subjected to the hot strong blast passing 45 through the converter. The temperature in this case also increases from the upper to the lower end of the converter cylinder, but this temperature is very much higher than in the first converter. As the ore passes 50 along the converter cylinder it will be subjected to a calcining heat which not only drives off any free moisture which may be present, but also drives off the combined moisture. The high temperature causes the 55 ore and any associated siliceous gangue to expand unequally and thus break open the lumps and expose this gangue. As the ore is thus tumbled around and subjected to the heat, the gangue will be loosened by the heat 60 and shaken loose by the tumbling action, and dried out so as to become very brittle, and this gangue is powdered by the tumbling action of the lumps against one another. This gangue so loosened and powdered will be picked up by the strong blast

passing through the converter and carried along with it, while the ore will continue downwardly toward the discharge end. The gangue will not only be shaken loose from the surface of the ore, but will also be shaken 70 out of the cracks and crevices in and around the ore, and this blast will also seek out the gangue in the cracks and crevices and separate it from the ore lumps, so that when the ore reaches the discharge end of the converter it will be freed of all of its clay gangue. It will therefore be seen that after the ore leaves the converter it will not only be entirely freed from its clay gangue, but also from all of its free and combined moisture, so that the ore will be in a dry and porous condition, brought about by the 75 cleaning out of the gangue and the expulsion of the combined moisture. Furthermore the cracking of the ore lumps and the 80 tumbling will free the siliceous gangue from the ore, so that while this siliceous gangue may not all be separated from the ore by the air blast, it will be loosened therefrom to enable it to be separated in the subsequent operation hereinafter to be described. The ore as it leaves the second converter is 85 at a cherry red heat, or at about  $1300^{\circ}$  F.

The ore as discharged from the second converter is sized in a sizing trommel to two 90 sizes, an undersize of one-half inch and less, and an oversize of one-half inch and over. This sizing takes place for two reasons. First, it is found that the oversize does not 95 contain very much siliceous gangue, and can therefore be conveniently and economically hand-picked, second, it is found that the subsequent magnetizing process and the subsequent magnetic separation can be performed more effectively if performed on an 100 undersize of one-half inch and less, although we have found that the magnetizing and magnetic separation can be performed on pieces which will pass through a one inch mesh. The oversize is cooled down by 105 sprays of water 75 and then discharged on a picking belt 73 where the ore is hand-picked.

The undersize from the sizing trommel 71 is passed directly to the third converter C. 115 This third converter is made as airtight as possible to prevent the entrance of outside air. The material is fed by the double valves, which exclude outside air, since these valves are so operated that one will be 120 always closed while the other is open. Entrance of air during the feeding of the ore is therefore prevented. A gaseous hydrocarbon atmosphere is maintained by feeding in crude oil under 150 lbs. pressure, and this 125 oil is fed in directly under the ore bed as it slides down the chute into the converter cylinder, so as to mix directly with the hot ore. This construction will also cause the ore sliding down over the end of the pipe to 130

keep the outlet clean and free. The oil forced into the converter cylinder will volatilize and form a dense and concentrated hydrocarbon atmosphere in the cylinder. 5 The upper end of the cylinder is of large diameter so as to furnish a large volume for the hydro-carbon gases to act on the material. The lower end of the cylinder, or rather the lower half, is reduced in diameter so as to form a small outlet, thereby preventing entrance of air. The swinging doors at the lower end of the converter cylinder will also keep out the air, and the large door is normally held closed while the lower or 10 small door only opens to let out the material. The material as it is discharged from the second converter B is at about 1300° F., and as discharged into the third converter C is at 1000° F. or over. The material is therefore maintained in the third converter at about 1000° F. and over 900° F., as it has been found that the temperature in this converter must be over 900° F. in order that the desired action may take place. The material is kept in the third converter C for 30 15 minutes or over. It has been found when treated as described, the ore as it leaves the converter is magnetic, *i. e.*, it is attracted by a magnet. The material as it leaves the converter is taken by a conveyer to a sizing trommel 116, and while being conveyed is subjected to the action of jets of water to cool the same. The material is sized to meet the varying requirements of magnetic separation and is then separated magnetically. 20 The material can be separated at as high a temperature as the magnetic separators will take it, but it will be found that it can be separated cold. 25 It is obvious that various changes may be made in the details of construction without departing from the spirit of this invention, and it is therefore to be understood that this invention is not to be limited to the specific 30 construction shown and described.

The process is fully described and claimed in our copending application, Serial Number 810,530, filed of even date herewith, while the magnetizing process *per se* is fully 35 described and claimed in an application of Robert W. Erwin, Serial Number 810,532, filed of even date herewith.

Having thus described the invention what is claimed is:

50 1. An apparatus for clearing ore of its gangue, comprising a converter receiving the ore and its gangue and having means for heating the material to preliminarily

render the gangue separable from the ore, a crusher receiving the material from the converter to preliminarily separate the gangue from the ore, a screen receiving the material from the crusher to preliminarily remove the gangue from the ore, a second converter receiving the oversize material from the screen and having means for heating the material, means coöperating with said second converter to tumble the ore therein and complete the separation of the gangue from the ore, and means for subjecting the ore and gangue in said second converter to a strong blast to remove the gangue from the ore.

2. An apparatus for clearing ore of its gangue, comprising a converter receiving the ore and its gangue and having means for heating and tumbling the material to preliminarily render the gangue separable from the ore, a screen receiving the material from the converter to preliminarily remove the gangue from the ore, a second converter receiving the oversize material from the screen and having means for heating the material, means coöperating with said second converter to tumble the ore therein and complete the separation of the gangue from the ore, and means for subjecting the ore and gangue in said second converter to a strong blast to remove the gangue from the ore.

3. An apparatus for clearing ore of its gangue, comprising a converter receiving the ore and its gangue and having means for heating the material and for subjecting the same to a blast, a crusher receiving the material from the crusher, a screen receiving the material from the crusher, and a second converter receiving the oversize material from the screen and having means for heating and tumbling the material and for subjecting the same to a blast to remove the gangue from the ore.

In testimony whereof we have hereunto affixed our signatures in the presence of these witnesses.

EDWARD F. GOLTRA.  
THOMAS S. MAFFITT.  
JESSE D. DANA.

Witnesses:

W. A. STINE,  
P. C. MAFFITT.

ROBERT W. ERWIN.

Witnesses:

HARRY ORR,  
FRANK CAMPBELL.